

## UNITED STATES PATENT OFFICE

2,038,572

PRODUCTION OF EMULSIFIABLE  
BITUMINOUS SUBSTANCES

Hans Klein, Mannheim, Germany, assignor  
to I. G. Farbenindustrie Aktiengesellschaft,  
Frankfort-on-the-Main, Germany, a corpora-  
tion of Germany

No Drawing. Application January 5, 1931, Serial  
No. 506,836. In Germany January 17, 1930

## 10 Claims. (Cl. 134—1)

The present invention relates to the production of emulsifiable bituminous substances, such as tars and the like.

I have found that bituminous substances, such as 5 tars, tar oils, petroleums, and petroleum asphalts and the like are obtained in an excellently emulsifiable state by incorporating substantially dry brown coal with the said bituminous substances. By substantially dry brown coal I hereinafter understand a brown coal having at the most a content of water of 3 per cent. Brown coal has the advantage, when employed in accordance with the present invention of having an excellent emulsifying action. The very simple 10 nature of its employment and its low cost are further advantages of brown coal.

Particularly emulsifiable products are obtained by adding the brown coal to the bituminous substances while heating, temperatures of from 100° to 200° C. being the most suitable. The mixing of the brown coal with the bituminous mass may be effected in a stirring vessel. The brown coal is preferably added in a finely divided state and dried before its employment. It is advantageous 15 to employ brown coal in such a state of subdivision that 90 per cent thereof pass through a sieve of 10000 meshes to the square centimeter. When the mixing is effected at elevated temperatures, however, the brown coal may also be used 20 in a moist state because the water evaporates during the mixing. The final content of water in the brown coal must, however, not exceed that above defined. The brown coal employed should preferably be rich in bituminous substances, and poor in humic acid; e. g. mid-German brown coal containing 5% of humic acid.

The resulting mixture is then emulsified in the manner already known, either as such or after the removal of any particles of coal which may have been deposited. The emulsification may for example be effected by stirring the mixture in a vessel provided with a stirring device and allowing a thin jet of water to flow into the mixture. The emulsifying action of brown coal is so marked that in many cases the simultaneous employment of alkaline reacting substances dissolved in the aqueous phase may be dispensed with. Even an addition of very small amounts of brown coal, as for example 0.5 per cent by weight of the emulsion, produces quite a marked effect, but 3 per cent by weight or even larger amounts should usually be added. With larger additions, the viscosity of the mixture is appreciably increased and this is frequently very desirable, as for example when working up very mobile tars. The

upper limits of the amounts of brown coal to be added is only determined by the desired final viscosity of the emulsion. Highly viscous products are for example obtained by adding 30 per cent by weight of brown coal to the emulsion, although even more may be employed.

The resulting emulsions may be employed as road constructional materials, for treating surfaces, for protective painting and the like.

The following examples will further illustrate 10 the nature of this invention, but the invention is not restricted to these examples. The parts and percentages are by weight.

## Example 1

15 300 parts of a mineral coal tar suitable for tarring the surface of roads are heated to 150° C. and 40 parts of ground brown coal containing 2 per cent of water are introduced during the course of half an hour while stirring. Before its 20 employment, the cooled mixture is emulsified with its own weight of water to give a 50 per cent emulsion in a cylindrical vessel provided with an inclined stirring device capable of being rotated at a high speed and having rings provided with 25 holes.

## Example 2

30 A mixture of 240 parts of mineral coal tar and 60 parts of petroleum asphalt is stirred at 160° C. with 50 parts of ground brown coal containing 2 per cent of water. Before its employment, the 35 cooled mixture is emulsified with its own weight of water in a cylindrical vessel provided with an inclined stirring device capable of being rotated at a high speed and having rings provided with holes.

What I claim is:—

1. The process of bringing a substantially water-free bituminous substance selected from a group consisting of tars, tar oils, petroleums and petroleum asphalts into a state in which it can be readily emulsified with water which consists in incorporating with said substance from 0.5 to 30% by weight of finely divided brown coal poor 45 in humic acid and containing not more than 3% of water.

2. The process of bringing a substantially water-free bituminous substance selected from a group consisting of tars, tar oils, petroleums and 50 petroleum asphalts into a state in which it can be readily emulsified with water which consists in incorporating with said substance from 0.5 to 30% by weight of finely divided brown coal poor in humic acid while heating to a temperature of from 55

- 100° to 200° C. until the content of water in the mixture is not more than 3%.
3. The process of preparing a water emulsion of a substantially water-free bituminous substance selected from a group consisting of tars, tar oils, petroleums and petroleum asphalts which consists in mixing said substance with from 0.5 to 30% by weight of finely divided brown coal poor in humic acid and containing not more than 3% of water and then mixing the composition thus obtained with water.
4. The process of preparing a water emulsion of substantially water-free mineral coal tar which consists in mixing with said tar about 13% of ground brown coal poor in humic acid while heating to a temperature of about 150° C. until the mixture contains not more than 3% of water and then incorporating with the resulting mixture about its own weight of water.
- 20 5. The process of preparing a water emulsion of a composition consisting of about 80% of substantially water-free mineral coal tar and about 20% of substantially water-free petroleum asphalt which consists in mixing with said composition about  $\frac{1}{6}$  of its weight of finely divided brown coal poor in humic acid while heating at a temperature of about 160° C. until the composition contains not more than 3% of water and then incorporating with the resulting mixture its own weight of water.
- 30 6. A composition suitable for emulsification with water consisting of a substantially water-free bituminous substance selected from a group consisting of tars, tar oils, petroleums and petroleum asphalts and from 0.5 to about 30% by weight of finely divided brown coal poor in humic acid and containing not more than 3% of water.
7. The process of preparing a water emulsion of a substantially water-free bituminous sub-

stance selected from the group consisting of tars, tar oils, petroleums and petroleum asphalts which consists in mixing said substance with from 3 to 30 per cent by weight of finely divided brown coal rich in bituminous substances and poor in humic acid and containing not more than 3 per cent of water and then mixing the composition thus obtained with water.

8. The process of preparing a water emulsion of a bituminous substance which comprises mixing with water a mixture of a substantially water-free bituminous substance selected from the group consisting of tars, tar oils, petroleums and petroleum asphalts with from 0.5 to 30 per cent by weight of finely divided brown coal poor in humic acid and containing not more than 3 per cent of water.

9. The process of preparing a water emulsion of a bituminous substance which comprises mixing with water a composition obtained by heating a mixture of a substantially water-free bituminous substance selected from the group consisting of tars, tar oils, petroleums and petroleum asphalts with from 3 to 30 per cent by weight of finely divided brown coal poor in humic acid until the content of water in the mixture is not more than 3 per cent.

10. The process of preparing a water emulsion of a bituminous substance which comprises mixing with water a composition obtained by heating a mixture of a substantially water-free bituminous substance selected from the group consisting of tars, tar oils, petroleums and petroleum asphalts with from 3 to 30 per cent by weight of finely divided brown coal rich in bituminous substances and poor in humic acid until the content of water in the mixture is not more than 3 per cent.

HANS KLEIN. 40